

Feb. 22, 1938.

L. E. CALKINS ET AL

2,108,847

ELECTRIC LAMP BULB

Filed April 8, 1937

FIG. 1



FIG. 2.



INVENTORS

Lyle E. Calkins, &  
Ormonde S. Levi

By *Dover & Dover*,  
ATTORNEYS

## UNITED STATES PATENT OFFICE

2,108,847

## ELECTRIC LAMP BULB

Lyle E. Calkins and Ormonde S. Levi, Toledo,  
Ohio, assignors to Save Electric Corporation,  
Toledo, Ohio, a corporation of Ohio

Application April 8, 1937, Serial No. 135,736

4 Claims. (Cl. 176—16)

This invention relates to bulbs for incandescent lamps, and particularly to those of the inside frosted type.

Inside frosted lamp bulbs have features of advantage in use over outside frosted or other types of light diffusing bulbs, and a considerable demand has resulted in the trade for lamps with such bulbs. In the past, difficulty has arisen in the inside frosting of such bulbs due to the frosting methods ordinarily employed, when applied to the inside of a bulb, effecting such a weakening of the bulb as to render it too fragile for commercial handling.

It has heretofore been found, however, that if a lamp bulb frosted on the inside in the usual manner is given a second or additional frosting treatment of lower degree than that to which it was first subjected, it becomes sufficiently strong for commercial handling, the strengthening action in such case being supposedly occasioned by the changing of the frosting pits or depressions from sharp angular to rounded form. It is further found, however, that while such treatment when first applied materially strengthens such bulbs against breakage, they weaken with age to such an extent that within a very few months the bulbs in many cases become so fragile as not to permit commercial handling without breakage.

The object of the invention is the production of an inside frosted electric lamp bulb of a strength suitable for commercial handling, which will not weaken with age, and which will, with a minimum of absorption of light, sufficiently diffuse the emitted light of the associated light source as to prevent any objectionable glare, thus giving maximum light emission, increasing the lamp life at designated efficiency and improving the ultimate lamp quality.

The invention is fully described in the following specification and illustrated in the accompanying drawing, in which—

Figure 1 is a side view, partly in section, of a lamp bulb embodying the invention, and Fig. 2 is a reproduction of a photomicrograph, enlarged 500 times, of the inside frosted surface of a bulb embodying our invention.

An electric lamp bulb embodying the invention is designated 1 in the drawing and has its interior surface 2 frosted by a chemical etching with such surface characterized by the presence of a multiplicity of acicular portions, by which term is meant elevations or projections of needle like or relatively long ridge like form running in different directions, as distinguished from a frosted

surface having a cellular, octahedral or lens like formation. Furthermore, the crests and crevices appear to be sharp or angular as distinguished from rounded. It is the presence of the acicular structure to which is largely attributed the strength of the inside frosted bulbs, as it is found that when such formation is absent the bulbs in general are too fragile for commercial handling. The frosted surface of our bulb is further characterized and is distinguished from the cellular frosted surface produced by the double treatment method described in U. S. Patent No. 1,687,510 to Pipkin by the absence of rounded crevices.

A most important feature in inside frosted bulbs of this character is that of strength to withstand breakage by impact, and in order to illustrate this feature the comparative strength tests hereinafter referred to were made on an ordinary type of bump tester such as shown and described in said Pipkin Patent No. 1,687,510. It is found, as stated in said patent, that inside frosted bulbs which show an impact strength of 7 or more on such tester, when made up into lamps, are sufficiently strong for commercial use.

The following strength readings, as determined by said tests, indicate for each set the average bump tester breakage point for twenty clear bulbs of each wattage taken at random from the same stock:

| Wattage                  | Clear | Inside frosted | Strength clear bulb 100% | 30 |
|--------------------------|-------|----------------|--------------------------|----|
| S-14 (10 watt)           | 87    | 17             | 10.5                     | 35 |
| A-17 (15 watt)           | 60    | 12             | 20                       |    |
| A-19 A5 (25 watt)        | 42    | 10             | 23.8                     |    |
| A-19 H2 (40 watt)        | 50    | 11             | 22                       |    |
| A-21 E4 (50 and 60 watt) | 55    | 12             | 21.8                     |    |
| A-21 G2 (75 watt)        | 61    | 13             | 21.3                     |    |
| A-23 (100 watt)          | 47    | 11             | 23.4                     |    |
|                          |       |                |                          | 40 |

The average shown for each of the above vertical sets of figures is 57.5 for the clear bulbs; 12.3 for the inside frosted bulbs, and 21.7 for the percentage of strength of inside frosted bulbs to clear bulbs. Tests further show that these inside frosted bulbs do not weaken with age, which is an important feature.

If, therefore, the average strength of clear bulbs to resist breakage by impact is 57.5, and the average minimum commercial strength requirement for inside frosted bulbs is 7, then it is apparent that inside frosted bulbs to resist breakage by impact should have an average strength of at least 12.15% of that of the clear bulb average. It is found that the strength of the frosted

bulbs varies with the extent to which the acicular projections or ridges are present.

Photometric tests were also made of certain wattage clear bulb lamps taken at random from regular stock and of similar lamps having our inside frosted bulbs to determine the maximum brightness of each. Twenty-five and sixty watt lamps were used for this purpose.

The average readings from these tests for the clear and inside frosted lamps of both wattages were as follows:

| 15 | Wattage | Maximum brightness clear | Maximum brightness inside frosted | Percent |
|----|---------|--------------------------|-----------------------------------|---------|
|    |         | 25                       | 173                               | 3.7     |
|    |         | 60                       | 605                               | 12.9    |
|    |         |                          |                                   | 2.1     |
|    |         |                          |                                   | 2.1     |

20 In making the above brightness tests, three lamps were used for each test and the bulbs therefore taken at random from regular stocks of the same make of clear and frosted bulbs, respectively, the frosted bulbs, before frosting, being as 25 nearly like the clear bulbs as possible to obtain.

The results of the above strength and photometer tests showed the average for the twenty-five watt clear bulbs to be strength—42, and maximum brightness—173. Lamps of twenty-five watt 30 frosted on the inside and embodying our invention showed strength—10, and brightness 3.7. Clear lamps of sixty watt showed average strength—55, and brightness—605. Sixty watt lamps frosted on the inside and embodying our 35 invention showed strength—12, and maximum brightness—12.9.

A further test was made to determine the lumen output for lamps having clear bulbs as compared to lamps having inside frosted bulbs embodying our invention, such tests showing the following lumen output readings:

| 45 | Bulbs                    | Clear   | Inside frosted | Percentage lumen output |
|----|--------------------------|---------|----------------|-------------------------|
|    |                          |         |                | clear bulb 100%         |
|    | A-17 (15 watt)           | 123.65  | 122.9          | 99.50                   |
|    | A-19 A5 (25 watt)        | 261.00  | 261.0          | 100                     |
|    | A-19 H2 (40 watt)        | 451.70  | 439.3          | 97.35                   |
|    | A-21 E4 (60 and 60 watt) | 746.70  | 742.8          | 99.50                   |
| 50 | A-23 (100 watt)          | 1521.00 | 1511.00        | 99.30                   |

55 In making the above lumen output tests, twelve bulbs were used in each of the tests and were taken at random from regular stock of the same make of clear and frosted bulbs, respectively, the frosted bulbs before frosting being as near like the clear bulbs as possible to obtain and such lamps each having a maximum brightness comparable to the above brightness readings.

60 The frosting solution preferably employed to produce on a lamp bulb an inside frosting having the characteristics above-pointed out may be divided into three parts, i. e., "A" the acid part, containing the acid and acid fluorides; "B" the crystalline part, containing the crystalline fluorides, sulphates and water, and "C" the binder part, containing molasses for increasing the consistency of the compound and giving it the requisite viscosity.

65 (A) Part "A" preferably comprises the following ingredients in substantially the proportions noted:

70 Ammonium acid fluoride----- 33 lbs. 3 oz.  
Hydrofluoric acid (approximately 75 60%)----- 10 liters

These materials are put into a drum of rubber, or other suitable acid resisting material, and rolled or agitated until complete solution takes place.

(B) Part "B" preferably comprises the following ingredients in substantially the proportions noted: 5

Sodium acid sulphate----- 11 lbs. 1 oz.  
Sodium fluoride----- 11 lbs. 1 oz.  
Water----- 6 liters 10

These ingredients are put into a rubber mill preferably containing bronze balls. This material is milled usually for at least three hours, or until it contains no lumps or unground materials. At 11 the beginning of the run, pressure is generated in the mill by the chemical reaction which takes place therein, and care should be taken to release this pressure. The mill should be watched for about fifteen minutes for this purpose. It is 20 preferable to use hot water to increase the solubility of the materials. It is found that the hotter the water the more speedy the action.

(C) Part "C" preferably comprises:

Molasses----- 12 liters 25

A commercial grade of molasses is used. The presence of the molasses in the solution retards the flow of the liquid by acting as a binder, and also retards, due to its viscosity, the rate of reaction of the solution. The change of viscosity of the molasses with temperature allows an easy method of controlling the etching action, and this is obtained by the application of heat to the outside of the bulb during the etching operation, as hereinafter described. It is found that by applying water to the outside of a bulb during the etching operation and by varying the time, the flow and temperature of the water, the formation of the crystalline structure of the 40 etched surface can be controlled.

When part "B" has been sufficiently milled, part "A" is added thereto and the whole is then preferably milled for at least half an hour or until a thorough mixing has taken place. This mixture 45 is then turned into a wooden tub and part "C" added, stirring well while adding. The solution which is now ready for use has a light brown creamy appearance and a consistency substantially equal to No. 10 motor oil. 50

The sodium fluoride contained in part "B" controls more or less the crystalline structure by stabilizing the viscosity of the solution. The sodium fluoride does not dissolve to any great extent and the fine particles thereof in suspension in the 55 solution form nuclei for crystal formation of ammonium, sodium and calcium silica fluorides (or fluosilicates). This crystalline structure is quite important in obtaining the desired strength characteristics of an inside frosted bulb. 60

There is also another use for the sodium fluoride in the solution. When sodium acid sulphate is mixed with sodium fluoride in aqueous solution, an exothermic reaction takes place, causing heat to be given off. This reaction forms some 65 free sulphuric acid, sodium sulphate, hydrofluoric acid and sodium acid fluoride along with sodium acid sulphate and sodium fluoride. All these substances are in a state of delicate chemical balance, and it is believed that this equilibrium 70 tends to stabilize the concentration of acid, sodium fluoride, sodium acid fluoride and sulphates in solution.

75 It is found that part "B", when used alone, will etch the glass, but the reaction is too slow for 75

commerical use, due to the low hydrofluoric acid content. When, however, parts "A" and "B" are thoroughly mixed together and part "C" added, a powerful frosting solution is obtained 5 and one which, when used in connection with the method hereinafter described, will produce an inside frosted bulb which is sufficiently strong against breakage to permit ordinary commercial handling, will effect a proper diffusion of light 10 emitted therefrom to prevent objectionable glare or brightness, and will have a greater lumen output with consequent higher initial rating than other inside frosted bulbs now made of which we are aware.

15 In practicing our invention in the inside frosting of a lamp bulb, the frosting solution above-described is first applied in stream or jet form under low pressure (about 1½ to 2 lbs.) up into the interior of the bulb, so that the stream strikes 20 the central top closed portion of the bulb, flows evenly down the sides and discharges from its lower open end. The solution is applied over a period of about ten seconds.

Immediately following the application of the 25 acid the bulb is subjected to an external hot water treatment to control the etching action of the acid adhering to the inner surface of the bulb. Hot water is caused to flow onto and down around the closed end of the bulb discharging 30 from its lower end, and the temperature of the water and time applied are important items in the etching operation in controlling the degree of etching and consequent acicular surface formation of the frost surface to produce the desired results. The temperature of the water 35 preferably should be approximately 63° C., and the water should be of sufficient quantity to completely cover the bulb. The time of application varies, depending on the bulb size, but for most 40 sizes the time is about ten seconds.

The bulb is next subjected to a thorough internal washing to entirely remove the etching acid therefrom and thus stop any further etching action. This washing is preferably accomplished 45 by discharging a stream of water under relatively high pressure (about 15 lbs.) up into a bulb from a rather small orifice (about  $\frac{1}{8}$  of an inch in diameter). For most satisfactory results the temperature of the water should be from 50° to 50 95° C.

After washing, the bulb is thoroughly dried preferably by directing hot air thereagainst, both inside and outside, and is then ready for use in

a lamp. The bulb may also be held over a flame to facilitate drying. Nothing new is claimed for the washing and drying operation.

This application is filed as a continuation in part of our application Serial No. 93,246, filed 5 July 29, 1936.

Having thus described our invention, what we claim as new, and desire to secure by United States Letters Patent, is:

1. A glass electric lamp bulb having its interior surface frosted by chemical etching so that the maximum brightness of an ordinary incandescent lamp comprising such bulb will be less than 20% of that of a like lamp with a clear bulb, said interior bulb surface being characterized by the presence of acicular portions to such an extent that the strength to resist breakage by impact is greater than 13% of that of a like clear bulb.

2. A glass electric lamp bulb having its interior surface frosted by chemical etching so that the maximum brightness of an ordinary incandescent lamp comprising such a bulb will be less than 15% of that of a like lamp with a clear bulb, said interior bulb surface being characterized by the presence of acicular portions to such an extent that the strength to resist breakage by impact is greater than 16% of that of a like clear bulb.

3. A glass electric lamp bulb having its interior surface frosted by chemical etching so that the maximum brightness of an ordinary incandescent lamp comprising such a bulb will be less than 15% of that of a like lamp with a clear bulb, said interior bulb surface being characterized by the presence of ridge-like elevations with sharp crests and crevices to such extent that the strength to resist breakage by impact is greater than 16% of that of a like clear bulb.

4. A glass electric lamp bulb having its interior surface frosted by chemical etching so that the maximum brightness of an ordinary incandescent lamp comprising such bulb will be less than 20% of that of a like lamp with a clear bulb, said interior bulb surface being characterized by the presence of a multiplicity of ridge-like elevations running in different directions to such extent that the strength to resist breakage by impact is greater than 13% of that of a like clear bulb.

50  
LYLE E. CALKINS.  
ORMONDE S. LEVI.